

## UNITED STATES PATENT OFFICE.

RUDOLF BRAUCKMEYER, OF GRUNBERG I/SCHLESIEN, GERMANY.

## METHOD OF DEGREASING RAW WOOL.

No Drawing. Application filed January 14, 1926, Serial No. 81,324, and in Germany May 25, 1925.

The invention relates to an improvement in or modification of the method of degreasing raw wool described in the specification of the prior Patent No. 1,521,624.

5 Numerous suggestions have been made for the degreasing of raw wool with the aid of organic solvents. The solvents suggested for the purpose, e. g. petrol, ether, carbondisulphide, tetrachlorcarbon, and so on, are those 10 which combine great degreasing capability with insolubility or poor solubility in water.

In contradistinction thereto a method is described in the specification of the said prior patent according to which raw wool is 15 greased by means of a mild grease solvent, namely acetone, as a result of which the wool is degreased to an extent which leaves in the wool the valuable capillary fat of the fibres within desired limits.

20 The present invention is based on the recognition of the fact that in order to carry out the de-greasing of raw wool and the like, the use of water soluble grease solvents is of considerable technical importance. In consequence of the great area of the fibrous material and the great spreading power of the organic solvent, considerable quantities of the solvent are retained in the material after completion of the extraction process. Even after 25 pressing the wool or subjecting it to centrifugal action, it contains in general more than 50% of its own weight in solvent. The removal of the solvent retained by the wool and its reextraction presents considerable technical difficulties. In consequence of the poor 30 heat conductivity of the wool for instance the supply of heat for evaporative purposes does not yield satisfactory results, while, for example, the passage therethrough of heated inert gases results in the production of very 35 highly diluted mixtures which do not permit of economical re-extraction of the grease solvent, for instance with the aid of absorption liquids or solid adsorption media.

40 Moreover, it has been observed that the freeing of the treated wool, from the solvent which is retained, by means of heat leads to injury of the fibres.

45 The use of water soluble grease solvents offers the great advantage that such solvents can be removed from the material in the simplest possible manner by the use of water (or aqueous solutions). It has already been suggested to remove insoluble grease solvents of 50 the kind mentioned at the commencement of this specification by means of water, but in

general only the solvent on the surface of the fibre is removed mechanically by the water, while more or less large quantities of the solvent remain within the fibres.

60 It has now been found to be of very great importance to treat the degreased fibre with water under such conditions that, on the one hand, the organic solvent is removed from within the fibre, and, on the other hand, a certain amount of water is taken up by the fibre. Experiments have shown that in using water-soluble solvents by simply washing or flushing the degreased wool with the water the solvent present therein is wholly removed, and at the same time water penetrates the interior of the fibre. Organic solvents 65 more difficultly soluble in water, for example, those which are soluble only in the ratio 1 to 10, or 2 to 10, in water, also come within the 70 scope of the present invention.

75 Moreover, the water soluble grease solvents to be used in accordance with the present invention and of which methyl alcohol is a 80 type, in consequence of their mild action compared with the solvents hitherto used, such as petrol, benzol or the like, afford the advantage already referred to in the specification of the prior patent, that the degreasing operation may be carried out in a regulatable 85 manner by which the valuable capillary fat is retained in the fibres in greater or smaller quantities.

90 In the specification of the said prior patent it has been indicated as a very desirable result to be sought that a fat content of about 2 to 5% should be retained in the fibres. It has now been found that degreasing can be carried further without danger which, of course, 95 is of advantage for subsequent dyeing of the fibres, if in the treatment of the fibres by water following on the extraction opportunity is afforded to the fibre to take up a certain amount of water by absorption, so as to replace the fat removed. As a result the fibre 100 is protected against damage even if the degreasing is carried further.

105 In the treatment of degreased wool with water the water-soluble potassium salts and potassium soaps are also extracted. The washing water containing the potassium compound may be used in the usual manner, for example, may be dried to provide potash or may be used for other purposes. Finally, treatment with water of the degreased wool offers the advantage that the 110 dirty constituents present in the wool are

removed without the addition of materials or compounds such, for example, as soda, which would tend to felt the fibre.

In carrying out my process it has been 5 found very advantageous to free from water the raw wool to be degreased, which generally contains 15 to 20% moisture before it is treated with solvent, for example, in such manner as to lower the water content of the 10 wool to about 2 to 3%. Preferably the water is removed by careful heating, for example, by means of hot air. As a result the wool fat hanging in lumps on the fibre is melted so that it is spread uniformly over the fibrous 15 material. In the subsequent extraction, in the first place the fat on the surface of the fibre is removed, while the capillary fat, which favourably affects the elasticity of the fibres, is retained. Moreover, by the removal 20 of the water from the wool prior to the extraction of the fat, the solvent action of the solvent is increased and a uniform degreasing of the wool ensured.

Finally, by the removal of the water from 25 the wool the advantage is obtained that the potassium salts and soaps do not pass into solution during the extraction of the fat, so

that after completion of the extraction process the latter can be removed and rendered suitable for further use, for example, by treatment to provide potashes.

It has also been found that the method of degreasing wool with the aid of mild water-soluble grease solvents can be applied with advantage to the degreasing of waste wool containing fat or mineral oil, as also for the removal of spinning oil from yarns and fabrics. Also in such circumstances preliminary removal of water and the treatment of the degreased material with water are to be recommended.

Claims:

1. Method of degreasing raw wool consisting in primarily freeing the wool from water leaving about 2 to 3% moisture in the wool, 45 then treating the wool with water-soluble mild grease solvent.

2. Method of degreasing raw wool consisting in primarily freeing the wool from water leaving about 2 to 3% moisture in the 50 wool, then treating the wool with methyl alcohol.

In testimony whereof I affix my signature.  
RUDOLF BRAUCKMEYER.